# EUROPEAN PATENT SPECIFICATION

(11) **EP 0 058 290 B1**
(45) Date of publication and mention of the grant of the patent: **04.07.1984**
(21) Application number: 81850237.9
(22) Date of filing: 08.12.1981
(51) Int. Cl.: E01C 7/26, E01C 11/16

(54) **Composition of a road surfacing mass**
Zusammensetzung einer Strassenbelagmasse
Composition d'une masse de revêtement routier

(30) Priority: 19.12.1980 SE 8009021
(43) Date of publication of application: 25.08.1982
(73) Proprietor: ROCKWOOL AKTIEBOLAGET, S-541 86 Skövde (SE); SKANSKA AKTIEBOLAG, S-211 02 Malmö (SE)
(72) Inventor: Andersson, Ingmar, S-414 62 Göteborg (SE); Nilsson, Nils-Olov, S-443 00 Lerum (SE); Karlsson, Elis, S-532 02 Axvall (SE); Sandberg, Ulrik, S-541 31 Skövde (SE)
(74) Representative: Avellan-Hultman, Olle

## Description

The present invention relates to a method of manufacturing and the use of a compression resistant and highly stable surfacing mass for heavy loaded surfaces, especially for high traffic and heavy loaded parts of streets and roads, the surfacing mass mainly comprising a stone material which is bound by an asphalt mass, as defined in the first part of claim 1.

The progress of the traffic in streets and roads, both as concerns the traffic intensity and the weight of the individual vehicles, has caused great demands on the stability of the road surfaces. This is to a special degree the case for exposed places like in front of traffic lights, at cross roads, at roundabouts etc., where surfaces masses comprising a stone material having asphalt as a binder often show to have insufficient stability.

A lack of stability in the surfacing mass comes to the effect that the mass is deformed especially due to the fact that the vehicle wheels depending on where unpacking of the surfacing mass provides lowered wheel tracks in the road way which necessitate an expensive maintenance. On the said exposed places the maintenance work further is difficult to carry out and causes traffic disturbances to a higher degree than normal road maintenance.

Attempts have been made to solve the problem involved in lack of stability by using so called skeleton masses i.e. masses in which the grain size in the stone material is graded, so that the load mainly is transferred over coarse stone grains which support each other. Thereby it has been possible to reduce the risk for settlings or packings, since the stone particles of the stone material have less possibility of regrouping the fewer stones take part in the transfer of load.

The demands on the properties of the binder, however, increases correspondingly, and in practice the character of the binder has become the most important factor for the stability of the surfacing mass. Thus it is important that the binder locks the stone particles effectively in their taken positions and prevents displacements or regroupings of the stone particles. The binding capacity may be increased by adding an increasing amount of binder in relation to the amount of stone material. In such case, however, there may be problems with so called asphalt run-off, what means that the hot asphalt during the mixing of asphalt with the stone material runs off the stone particles, what both counteracts the intension of increasing the amount of binder, and also causes problems at storing and transport. The stability of the surfacing masses is not substantially increased, possibly depending on the so called cold flow of the asphalt.

Attempts have been made to solve these problems by adding a fine grain filler material, but the result does not seem to have been satisfactory. Obviously the skeleton principle partly gets lost when adding a fine grain filling material.

Attempts have been made to solve the problem by adding asbestos-fibres, but asbestos-fibres do not seem to give the skeleton masses sufficient increase to stability for the amounts which can be used technically. The reason for this probably is the tendency of the asbestos-fibres to hook to each other thereby forming larger aggregates. The knowledge of the health risk with asbestos-fibres further makes it out of question to use asbestos for road covering.

In the Swedish patent 211,163 a surfacing material is described which comprises mineral fibres having a diameter of between 5 and 15 ,um, also the suggested coarse mineral fibres have proved not to be useful. Probably such fibres tend to orientate parallelly to the stone surfaces of the asphalt-stone mass and thereby to the plane of the binder film. Therefore they hardly contribute to the stability of the skeleton mass. None of the suggested methods has come to any substantial practical use.

The above mentioned problems are solved by the method according to the characterising part of claim 1.

Surprisingly it has now shown that an addition of a mineral fibre material having a small fibre diameter preferably a fibre material having an average diameter which is less than 5 pm and in which the particles are even distributed in the asphalt mainly as separate fibres strongly reduces or eliminates the above mentioned cold flow problem of the binder or the asphalt. Thereby a binder phase is obtained giving the ready surfacing mass substantially increased stability as compared with previously known surfacing masses without giving a too high viscosity at mixing temperatures for a quick and careful mixing. The increased stability depends on an increased strength of the binder which probably depends both on the increased thickness of the binder film around the stone grains and also that the added fibre material, which is evenly distributed as separate fibres in the asphalt, as a reinforcing action.

As fibres may be used many different types of material provided that the fibres do not melt in the asphalt which during the mixing with the stone material is kept at a temperature of 140-170°C or preferably 150-160°C and also supposing that the fibres are sufficiently stiff and maintain at least a substantial stiffness in the hot asphalt. It has shown that a particularly suitable material is mineral fibres, for instance stone fibres, viz. fibres manufactured by melting stone like diabas and a subsequent fibrating of the melted stone.

As mentioned above the average fibre diameter should be less than 5 ,um. When the average fibre diameter is less than 1 ,um the favourable effect of the fibres is obviously reduced, probably in that the thin fibres irrevocably are shortened substantially during the mixing operation. The average fibre diameter consequently should be between 1 pm and 5 ,um. For giving the intended effect the fibres should be added in an amount by weight of 0.5 and 20% as calculated on the weight of asphalt, what corresponds to about 0.03-1.2% by weight of the ready surfacing mass.

It is important that the fibres are not present in the form of tots or other baked together aggregates. This can be avoided by a correct admixing techniques. For facilitating the distribution of the fibres and for avoiding formation of tots and for providing an optimum wetting of the fibre surfaces with asphalt it may be advantageous to treat the surfaces of the fibres with some suitable substance. For this purpose all kinds of non-polar compounds can be used, or instance wetting agents like catjonic tensides in the form of tertiary or quartery ammonium compounds.

It is also advantageous that the fibres are as dry as possible when being admixed in the asphalt, and for obaining an effect similar to the above mentioned treatment with a wetting agent it may be advantageous to dry the fibres before mixing the fibres into the asphalt or surfacing masses so the main part of the water molecules normally absorbed to the surfaces of the fibres are removed.

The admixing of the fibres may be made by adding the fibres to the stone material before the asphalt is admixed therein or the fibres may be admixed into the ready asphalt-stone mass. An especially good effect, however, is obtained if the fibres are mixed with the asphalt mass before adding said mass to the stone material. This facilitates the mixing and the equilizing of the fibres, and the mixing of the fibre material and the asphalt material can be made indulgently to the fibres so that the fibres are not broken.

Uneven and tot free distribution of the fibres in the asphalt is further favourized if the asphalt in connection to the admixing of the asphalt is heated, for instance to 20-40⁰C over the temperature of about 150-160°C which the asphalt material and the stone material are mixed, whereupon the asphalt-fibre mixture is cooled to said temperature and is admixed in the stone material. The temperature increase reduces the viscosity of the asphalt and thereby facilitates a homogenous and indulgent admixing of the fibre material, and further the wetting of the fibre surfaces is facilitated at the said increased temperature, and the dispersing of the fibres in the asphalt is made quickly and effectively.

For estimating the effect of the admixing of the fibre material on the stability of the asphalt surfacing a number of fibre masses were made according to three different methods and within each group with different amounts of admixed fibre material.

### Example 1

In a mixing apparatus for asphalt masses was introduced 1,100 kg of a stone material having a predetermined distribution of the average grain size. The stone material was heated to 160°C, and to the stone material was added 5,8 kg of a mineral fibre material named "INORPHIL 057"a by the manufacturer Rock- wool AB which material has an average fibre diameter of 3 pm and in which the main parts of the fibres are within the area of between 1 and 5 um.

For characterizing the fibre length there are no acceptdble direct method. Therefore preferably the so called thickening number (n_{f}) is defined, which is calculated by the formula in which n is the viscosity of a slurry of 1.5 g dry fibre in 200 ml ethyleneglycol at 20°C and in which ηₒ is the viscosity of the same ethyleneglycol without fibres likewise at 20°C and measured with the same equipment, viz. a Brook- field viscosimeter having a spindle LV1 or corresponding. For "INORPHIL 057" the thickening number is 1.0-5.0.

To the mixture of stone material and fibre material was admixed 195 kg asphalt. After finished mixing the mass was taken out and the stability and postpacking tendency was measured. This is made according to the following method:
A predetermined amount of the surfacing mass is put into a frame of angle iron 80x80 mm. The frame has a length of 2,000 mm and a width of 400 mm and is lying on a concrete floor. The surfacing mass is isolated from the concrete floor by an aluminum foil.

After two days (48 hours) at about 18°C the height position for eight different points along the center line of the frame is measured in relation to the frame. The mutual distance between the points is 200 mm. The measuring points are provided by a circular disc having a diameter of 20 mm which is put on the measuring point.

Thereafter a cylindric roll having a length of 100 mm and a diameter of 350 mm and loaded by 2000 N (200 kg) is rolled five times in both directions over the mass along the center line. The height of the above mentioned measuring points are once again noted and the difference to the original height is utilized as a measurement on the post-packing of the mass. The values are compared with corresponding values of post-packing of a normal mass, whereby the following value bases are used:
"Normal", 0.8-1.2 times the deformation of the normal mass;
"Slight postpacking" 1.2-1.6 times the deformation of the normal mass;
"Obvious postpacking", more than 1.6 times the deformation of the normal mass.

In Example 1 the mass had an obvious post- packing tendency.

### Examples 2-6

Example 1 was repeated with the same type of mineral fibre but of different length for the admixed fibre. The amount of admixed fibres and the results are made account for in the following table.

### Examples 7-9

In these examples the mineral fibre material was admixed in the hot asphalt before the asphalt-mineral fibre mixture was added to the stone material and was mixed therewith. The results are shown in the table.

### Examples 10-12

In these Examples the asphalt was heated to 190°C, whereupon the mineral fibre material was admixed in the asphalt, the asphalt-mineral fibre mixture was cooled to 160°C and was admixed in the stone material. The results are shown in the table.

### Example 13

In this Example was used a comparative mineral fibre having an average diameter of 6-8 gm, but for the rest the method according to Example 1 above was repeated.

### Example 14

In this case was used the same type of mineral fibre as in Examples 1-12 above, but in order to determine the effect of the fibre length, the fibre material was ground, whereby the fibre material obtained a thickening number of 0.2.

From the above table it is evident that even the least amount of admixed fibre has a substantially effect on the stability and the post- packing tendency of the material. When adding 0.3% by weight of the fibre material of the indicated type there is an obvious post-packing tendency according to Example 1, and according to Example 7 there is a slight post-packing tendency. In case that about 0.5 or a higher percentage of mineral fibre is admixed a normal post-packing is obtained. This is especially the case when the admixing follows according to Examples 7-9 and 10-12 respectively. The table also shows that coarse fibre according to Example 13 gives an obvious post-packing tendency and that also fibres having an average diameter of less than 5 pm give substantially better property than the coarser fibres. The table also shows that the fibre length has some effect in that the ground fibre material is used in Example 14 gives an obvious postpacking tendency.

In the accompanying drawing is diagrammatically shown an apparatus for manufacture of a surfacing mass according to the invention. In a tank 1 having heating coils 2 an asphalt mass 3 is heated to normal mixing temperature or, as mentioned above, to a temperature which is 20-40°C above said mixing temperature. By means of a pump 4 the hot asphalt is batchwise pumped over to a mixing container 5 which is formed with a stirring device 6, and to which mineral fibres are batchwise added from a container 7. After stirring to provide a homogenous mixture the asphalt fibre mass is pumped through a heat exchanger 9 by means of a pump 8, in which heat exchanger the temperature of the asphalt fibre mixture is adjusted to correct temperature for being mixed with the stone mass. In case the mixture of asphalt and mineral fibre is made at elevated temperature the mass is cooled, and if the mixture is made at the normal admixing temperature at for instance 150-160C and some cooling may have occurred during the handling of the mass some adjustment for increasing the temperature may be necessary.

The stone material is heated in a container 10 having heating means 11 and from there the stone material is batchwise transferred to a rotating mixer drum 12. The mass coming from the mixing container 5 for asphalt and mineral fibre is likewise pumped batchwise through the heat exchanger 9 to the mixer drum 12 and is mixed with a stone material with the same temperature for the two phases.

As previously mentioned the mineral fibre material can be supplied directly from the mineral fibre container 7 to the mixer drum 12 for asphalt and stone material, and in this case, of course, the asphalt is also pumped directly from the asphalt tank 1 to the mixture drum 12.

It is to be understood that the above specification and the apparatus illustrated in the drawings are only illustrating examples, and that many different modifications may be presented within the scope of the appended claims.

## Claims

1. Method of manufacturing a compression resistant and highly stable surfacing mass for heavy loaded surfaces and mainly comprising a stone material which is bound by an asphalt mass, in which the asphalt (3) is heated to a temperature at least corresponding to the recommended temperature for mixing the asphalt with the stone material, and concurrently herewith the stone material is heated to the recommended mixing temperature, the heated asphalt and the heated stone material are mixed to a homogenous mixture in the proportions 15-25 parts by weight of stone material per part by weight of asphalt, characterized in that an amount of 0.5-20 percent by weight of a fibre material calculated on the amount of asphalt and having an average fibre diameter of between 1 pm and 5 pm and of a type which is not dissolved or softened to a substantial degree in the hot mass is added during the handling of the surfacing mass.

2. Method according to claim 1, characterized in that the fibre material is a mineral fibre, and in that the fibre material is added to the heated asphalt and is mixed to a homogenous mass of fibres dispersed in the asphalt before the asphalt-fibre mass is admixed in the stone material.

3. Method according to claim 2, characterized in that the asphalt is heated to a temperature about 20--400C above the recommended mixing temperature for the asphalt-stone mass before the fibre material is added to the asphalt or before the mixture of asphalt and fibre material is added to the stone material.

4. Method according to any of claims 1, 2 or 3, characterized in that the fibre material is treated with a wetting agent like a catjonic tenside before the fibre material is added to the asphalt.

5. Method according to any of claims 1, 2 or 3, characterized in that the fibre material is dried completely before the addition thereof to the asphalt material.

6. Method according to any of claims 2-5, characterized in that the asphalt fibre mixture is cooled to the recommended admixing temperature before mixing the asphalt-fibre mass with the stone material.

7. Method according to any of the preceding claims, characterized in that the added fibre material is chosen among a group of material having a thickening number n_{f} of between 1.0 and 5.0.

8. The use of a surfacing mass manufactured according to any of claims 1-7 as a surfacing for streets and roads, especially a surfacing at cross streets, in front of stop lights, in traffic roundaways and other strongly frequented traffic points.

## Revendications

1. Procédé de production d'une masse de revêtement résistant à la compression et très stable pour surfaces lourdement chargées et comprenant principalement un matériau pierreux qui est lié par une masse d'asphalte, dans lequel l'asphalte (3) est chauffé à une température correspondant au moins à la température recommandée pour mélanger l'asphalte au matériau pierreux, et, simultanément, le matériau pierreux est chauffé à la température recommandée de mélange, l'asphalte chauffé et le matériau pierreux chauffé sont malaxés en un mélange homogène dans les proportions de 15-25 parties en poids de matériau pierreux par partie en poids d'asphalte, caractérisé en ce qu'une quantité de 0,5-20% en poids d'une matière fibreuse, calculée sur la quantité d'asphalte et ayant un diamètre moyen de fibre entre 1 µm et 5 ,um et d'un type qui n'est pas dissous ou ramolli à un degré substantiel dans la masse chaude, est ajoutée pendant la manipulation de la masse de revêtement.

2. Procédé selon la revendication 1, caractérisé en ce que la matière fibreuse est une fibre minérale, et en ce que la matière fibreuse est adjoutée à l'asphalte chauffé et est malaxée en une masse homogène de fibres dispersées dans l'asphalte avant que la masse asphalte-fibres soit ajoutée au matériau pierreux.

3. Procédé selon la revendication 2, caractérisé en ce que l'asphalte est chauffé à une température d'environ 20-4.0°C au-dessus de la température recommandée de mélange pour la masse asphalte-pierres avant que la matière fibreuse soit ajouté à l'asphalte ou avent que le mélange d'asphalte et de matière fibreuse soit ajouté au matériau pierreux.

4. Procédé selon l'une quelconque des revendications 1, 2 ou 3, caractérisé en ce que la matière fibreuse est traitée avec un agent mouillant analogue à un agent tensio-actif cationique avant que la matière fibreuse soit ajoutée à l'asphalte.

5. Procédé selon l'une quelconque des revendications 1, 2 ou 3, caractérisé en ce que la matière fibreuse est séchée complètement avant d'être additionnée à la matière asphaltique.

6. Procédé selon l'une quelconque des revendications 2-5, caractérisé en ce que le mélange d'asphalte et de fibres est refroidi à la température recommandée de mélange avant que la masse asphalte-fibres soit mélangée au matériau pierreux.

7. Procédé selon l'une quelconque des revendications précédentes, caractérisé en ce que la matière fibreuse ajoutée est choisie dans un groupe de matières ayant un indice d'épaississement n_{f} entre 1,0 et 5,0.

8. Utilisation d'une masse de revêtement produite selon l'une quelconque des revendications 1-7 comme revêtement de rues et routes, en particulier un revêtement de carrefours en avant de feux de circulation, de voies de circulation giratoires et d'autres points de circulation très fréquentés.

## Patentansprüche

1. Verfahren zur Herstellung einer druckbeständigen und hochstabilen Oberflächenbelagmasse für hoch-belastete Oberflächen die hauptsächlich ein durch eine Asphaltmasse gebundenes Steinmaterial enthält, wobei dem der Asphalt (3) mindestens auf die für das Mischen des Asphaltes mit dem Steinmaterial empfohlenen Temperatur und gleichzeitig hiermit das Steinmaterial auf die empfohlene Mischungstemperatur erhitzt und der erhitzte Asphalt und das erhitzte Steinmaterial in einem Verhältnis von 15-25 Gewichsteilen Steinmaterial pro Gewichtsteile Asphalt zu einer homogenen Mischung vermischt werden, dadurch gekennzeichnet, daß ein Fasermaterial, das während der Herstellung der Oberflächenbelagmasse durch die heiße Masse nicht wesentlich gelöst oder aufgeweicht wird, in einer Menge von 0,5-20 Gewichtsprozenten bezogen auf die Asphaltmenge und mit einem mittleren Faserdurchmesser zwischen 1 ,um und 5 ,um zugesetzt wird.

2. Verfahren nach Anspruch 1, dadurch gekennzeichnet, daß das Fasermaterial eine Mineralfaser ist und daß das Fasermaterial dem erhitzten Asphalt zugesetzt und mit diesem zu einer homogenen Masse von mit gleichartiger Faserverteilung vermischt wird bevor, die Mischung aus Asphalt und Fasermaterial dem Steinmaterial zugemischt wird.

3. Verfahren nach Anspruch 2, dadurch gekennzeichnet, daß der Asphalt auf eine ungefähr 20-4.0°C höhere Temperatur als die empfohlene Mischungstemperatur für die Asphalt-Stein-Masse erhitzt wird, bevor das Fasermaterial dem Asphalt oder bevor die Mischung Asphalt-Fasermaterial dem Steinmaterial zugesetzt wird.

4. Verfahren nach Anspruch 1, 2 oder 3, dadurch gekennzeichnet, daß das Fasermaterial mit einem Benetzungsmittel, wie einem kationischem Tensid, behandelt wird, bevor das Fasermaterial dem Asphalt zugesetzt wird.

5. Verfahren nach einem der Ansprüche 1, 2 oder 3, dadurch gekennzeichnet, daß das Fasermaterial vor dem Zusetzen zum Asphaltmaterial vollständig getrocknet ist.

6. Verfahren nach einem der Ansprüche 2 bis 5, dadurch gekennzeichnet, daß die Asphalt-Faser-Mischung auf die empfohlene Zumischtemperature abgekühlt wird, bevor die Asphalt-Faser-Masse mit dem Steinmaterial gemischt wird.

7. Verfahren nach einem der vorhergehenden Ansprüche, dadurch gekennzeichnet, daß das zugesetzte Fasermaterial aus einer Materialgruppe mit einer Eindick-Zahl n_{f} zwischen 1,0 und 5,0 ausgewählt wird.

8. Verwendung der nach einem der Ansprüche 1-7 hergestellten Oberflächenflächenbelagmasse als Straßenbelag, insbesondere als Oberflächenbelag an Kreuzungen, vor Ampeln, in Kreisverkehrbereichen und an anderen stark frequentierten Verkehrspunkten.
